

Oct. 22, 1935.

A. J. L. MORITZ

2,018,565

SPINNING PROCESS AND APPARATUS

Original Filed Nov. 2, 1931

Fig. 2.



Fig. 3.



Fig. 1.



Adrianus J. L. Moritz,  
INVENTOR

BY *Alvin F. Knight.*  
ATTORNEY

## UNITED STATES PATENT OFFICE

2,018,565

## SPINNING PROCESS AND APPARATUS

Adrianus J. L. Moritz, Enka, N. C., assignor to  
American Enka Corporation, Enka, N. C., a cor-  
poration of Delaware

Original application November 2, 1931, Serial No.  
572,670. Divided and this application January  
28, 1935, Serial No. 3,863. In Germany March  
14, 1931

## 5 Claims. (18-8)

This application is a division of my application  
Serial #572,670, filed November 2, 1931.

The present invention relates to a process and  
apparatus for rendering the dyeing properties of  
5 filaments uniform.

The invention is particularly designed for use  
in the spinning of artificial silk filaments and  
the winding of such filaments upon the spool  
or bobbins.

10 It has been ascertained that in the ordinary  
method of spinning according to the spool and  
roller process wherein the freshly spun filaments  
are wound with approximately constant or uni-  
form tension that considerable difference in dye-  
15 ing properties may be observed between the first  
and the last layers of the filaments upon the  
bobbins. Experiment has shown that these dif-  
ferences are due in large part to the fact that  
the uppermost, softly stratified layers of fila-  
20 ments, after the washing can shrink consider-  
ably during the drying, while the lower layers,  
for the most part lying against the hard core of  
the spool or roller cannot shrink to the same  
extent.

25 It is an object of the invention to overcome  
this defect to a great extent by increasing the  
tension upon the filaments as the thickness of a  
bobbin or spool increases so that the outermost  
20 layers of filaments upon a wound spool are wound  
relatively taut.

30 It is a further object of the invention to pro-  
vide a simple and easily manufactured article  
which can be attached to the machine at present  
in use and which will insure uniform density  
35 of the yarn bcd' at the same time, while a con-  
siderable uniform braking or initial tension is  
imparted to the filaments running on the bobbin,  
and will also increase in a certain predetermined  
40 measured degree the winding tension as the spool  
becomes thicker. Due to this fact it is unneces-  
sary to employ any complicated device to prac-  
tice the process.

45 It is also an object of the present invention to  
make use of the traversing filament guide itself  
for producing the tension upon the filaments.  
However, it is obvious that the tension upon the  
filaments running upon the spool or bobbin can  
50 be increased by means of numerous mechanisms  
and the following exemplification is designed  
merely to serve as an example, and is not to be  
construed in a limiting sense.

55 With these and other objects in view as will  
become apparent as the description proceeds, the  
invention consists in the steps and combination

of elements set forth below and shown in the  
drawing, in which

Figure 1 is a side view of an embodiment of the  
invention, diagrammatically shown,

Figure 2 is a similar illustration of the mech- 5  
anism shown in Figure 1 when viewed in front  
thereof, and

Figure 3 is a modified form of traversing mech-  
anism for supporting the thread guide.

In the drawing like reference characters refer 10  
to similar parts throughout.

Referring to the drawing, the filament or  
thread guide 2 is attached in any desired manner  
to the guide support 1. The guide 2 is provided  
with two friction rods or friction points 3 and 4 15  
over which the filament 5 is guided in zigzag  
manner to the spinning spool or bobbin 6.

As is apparent from the showing in Figure 1,  
due to the position of the brake rods 3 and 4 and  
the manner in which the filament is guided at an 20  
angle about the brake rods and also due to the  
position and rotational direction of the spinning  
spool or bobbin, the angle A will become smaller  
with the increasing spool winding and thus the  
25 tension of the filament running upon the spool  
or bobbin is accordingly increased.

The traverse mechanism may in this instance  
be constructed as a slide device as shown in Fig-  
ures 3 or as a suspension device as shown in Fig-  
ures 1 and 2. In addition to the means above de- 30  
scribed for gradually increasing the tension  
placed upon the filament rising from the spin-  
ning bath 7, the filament between the traverse  
filament guide and the spinning nozzle 8 can also  
35 be tensioned and stretched in any other manner  
either by a more or less lengthy immersion pas-  
sage or by additional filament guides which may  
be positioned within or without the spinning  
bath 7. It is also obvious that filament guide 2  
40 may be positioned as desired whereby different  
degrees of tension may be imposed upon the fila-  
ments.

According to the embodiment of the invention  
shown in Figures 1 and 2, the last brake rod 4  
which is interposed directly before the winding 45  
spool or bobbin, is bent to a peculiar hook shape  
as shown more particularly in Figure 2. Due to  
the hook shape the filaments in the cross or trans-  
verse movement will remain approximately at  
the same point upon the filament guide member 50  
and a properly calculated crossing of the filament  
may thus be obtained. It is of course, also obvi-  
ous that the filament guide may be constructed  
in a variety of forms to accomplish the functions  
and results desired as set forth above. 55

Thus, according to Figure 3 the filament guide may be attached in a vertical position upon the guide support 9 and this form of the invention is particularly suitable for a slide traverse mechanism in which a large number of horizontally mounted filament guide supports are used.

As above mentioned, it is possible to use many constructional forms of filament guides for securing the results desired, wherein application of the same will successfully facilitate performance of the above described method.

What I claim is:

1. A process for the manufacture of artificial silk having substantially uniform dyeing qualities throughout all parts of a wound package which comprises ejecting a cellulosic solution from a spinnerette into a spinning bath, tensioning the thus formed filaments by leading the same over guides in advance of a collecting device, and gradually increasing the said tension during the formation of the package to compensate for different degrees of contraction normally occurring which would otherwise cause non-uniformity in the dyeing quality of the filaments in different parts of the package.

2. A process for the manufacture of artificial silk filaments having substantially uniform dyeing qualities throughout all parts of a wound package which comprises gradually increasing the tension on the filaments as they are ejected from a spinnerette into a spinning bath and collected at a collecting device, and controlling this increasing tension by passing the filaments over tension guides in such a manner that the angle of contact of the filaments with the tension guides decreases as the winding proceeds to compensate for variations in the filaments which would otherwise cause non-uniformity in the dyeing qualities of the filaments in different parts of the package.

3. A process of manufacturing artificial silk comprising ejecting a cellulosic solution from a

spinnerette into a spinning bath, passing the newly formed filaments from the bath to a point of collection and there winding the filaments into package form in which there is a relative difference in resistance to contraction between the inner and outer layers thereof, applying tension to the newly formed filaments during their passage to the point of collection, thereby to stretch the same, and gradually increasing the tension on the filaments as the winding operation progresses.

4. A process for the manufacture of artificial silk having substantially uniform dyeing qualities in which the filaments are formed into a package wherein there is a relative difference in resistance to contraction between the inner and outer layers thereof comprising ejecting a cellulosic solution from a spinnerette into a spinning bath, passing the newly formed filaments from the bath to a point of collection and collecting the filaments in package form in which a relative difference in resistance to contraction exists between the inner and outer layer thereof, applying tension to the newly formed filaments during their passage to the point of collection thereby to stretch the same, and gradually changing the tension on the filaments as the winding operation progresses to effect a gradually increased stretching of the filaments toward the end thereof which is subject to the least resistance to contraction in the formed package.

5. An apparatus for the manufacture of artificial silk filaments and the like which comprises means for collecting the filaments at a substantially constant rate and means located in advance of a collecting device for effecting a progressive increase in tension on the filaments during their passage to the collecting device, whereby when a package is formed and dried it will have substantially uniform dyeing properties throughout all parts thereof.

ADRIANUS J. L. MORITZ.